

## UNITED STATES PATENT OFFICE

VICTOR L. SODERBERG, OF DETROIT, MICHIGAN

## METHOD OF FRACTIONALLY PLATING OBJECTS

No Drawing.

Application filed May 7, 1927. Serial No. 189,744.

It is frequently desirable to electroplate parts of an object with chromium while other parts, on which metal will be deposited when the object is subject to the plating process, should be left unplated. For example, the backs of reflectors or surfaces of other objects that are ordinarily hidden in use may be left unplated. Also, areas to which solder is to be applied, or which are to be painted or 10 enamelled, should be left free of plating. Screw threads, in many instances, and finished surfaces adapted to make fine fits or form elements in joints or parts of tools and dies should be left in a virgin state. When 15 such surfaces are plated with chromium there is a waste of energy and material as well as, in most instances, an actual objection to the presence of plate.

The object of the present invention is to 20 produce a simple and novel method of plating with chromium only those areas on which plating is desired, even though there are adjacent or other areas which, in ordinary practice, would become plated.

I have found that if those areas that it is 25 desired to leave free from plate and which would otherwise receive a deposit of metal during the plating process, are covered with an electrically-insulating substance insoluble 30 in the plating bath, the covered surfaces will not become plated in the subsequent electro-deposition process. The protective insulating covering should preferably, however, be soluble in removers, that is, compounds of 35 some kind for removing them after the plating process is completed.

Any cheap nitrocellulose lacquer may be 40 used advantageously for the protective covering, as will also liquid glass compounds as for example so-called "water glass", in the process of chromium plating. Other substances may also be used, provided that they will not harm or throw anything of a harmful, poisonous or detrimental nature into the 45 chromium plating solution.

The covering of large areas is particularly 50 advantageous in chromium plating where heavy currents are required, as the currents are thereby localized in the areas requiring plating and much less current is required.

than would be the case if no protective coating were employed. Furthermore, in the present state of development of the art of chromium plating, if the anodes are so placed as largely to concentrate the current in the 55 areas which it is desired to plate, the other areas often become etched due to the inefficiency of the chromium bath. The protective insulating coating prevents such etching and a higher efficiency of the specially-placed 60 anodes results. Again, where the currents are localized as far as practicable, there will still be more or less plating on the areas which should be left unplated, such plating being 65 streaky and uneven; this objection being also overcome by the use of the protective covering.

After the areas that are to be left unplated have been properly covered with the insulating material and preferably after the insulating material has dried, the plating process 70 is carried on in the usual way, with the result that the unprotected areas receive a deposit of metal, whereas the insulating material prevents any plating of the surfaces covered thereby. 75

When the plating operation has been completed the insulating material may be removed or not, depending on the nature of the work and the uses to which it is to be 80 put.

## I claim:

The process of treating an object so as to 85 electroplate with chromium only a portion of the surface on which chromium would normally be deposited during a plating operation, which consists in covering with nitrocellulose lacquer those portions of the object that are to remain unplated, and then placing the object in any usual or suitable bath 90 adapted for chromium plating and completing the plating process in any usual or suitable manner.

In testimony whereof, I sign this specification.

VICTOR L. SODERBERG.

95